

## UNITED STATES PATENT OFFICE

2,478,975

## TREATMENT OF HOSIERY

Albert Mellor, Ralph James Mann, Donald Finlayson, and Albert William Morledge-Hadfield, Spondon, near Derby, England, assignors to Celanese Corporation of America, a corporation of Delaware

No Drawing. Application October 9, 1945, Serial No. 621,379. In Great Britain October 30, 1944

5 Claims. (Cl. 117—56)

1

This invention relates to textile materials and especially to light textile fabrics and particularly light knitted fabrics of the kind of which hosiery is constituted.

Knitted hosiery of silk has long been highly valued on account of its apparent transparency or "sheerness" when on the wearer and the uniformity obtainable in respect of this and other properties, for example lustre. It is very difficult if not impossible to secure these properties in the same degree in hosiery and other textile fabrics made from less expensive yarns of cotton or artificial filaments, for example those of regenerated cellulose. These artificial filaments include those obtained from viscose or from cuprammonium cellulose solutions and those obtained by saponifying cellulose ester filaments substantially completely.

We have now found that a great improvement in sheerness and uniformity of appearance of textile materials and especially of light weight fabrics, for example knitted or woven fabrics having a weight of less than 2 ounces per sq. yard, can be secured by finishing them with a small proportion of a drying oil for example linseed oil or tung oil. After impregnation the material can be hung in the air so as to dry the oil by oxidation.

Preferably, more particularly in the case of cellulose materials, the textile material is first subjected to the "clarifying" treatment described in our co-pending U. S. application Serial No. 621,378, of even date. This treatment involves subjecting the materials to the combined action of water and hydrophobe liquid. By this preliminary treatment it is possible to enhance very considerably the desired effects. The hydrophobe liquid includes aliphatic or aromatic hydrocarbons, for example, benzene, toluene, xylene, solvent naphtha or light fractions of petroleum. Halogenated hydrocarbons, such as, for example, carbon tetrachloride or perchlorethylene can also be used. Furthermore, difficultly volatile or substantially non-volatile hydrophobe organic compounds can be employed, such as, for example, dimethyl phthalate, diethyl phthalate, di-(methoxyethyl)-phthalate and methylcyclohexanol, all of which are liquids of low volatility, the esters of phthalic acid being substantially non-volatile.

The treatment of the invention is of especial value in connection with hosiery made from yarns of regenerated cellulose filaments and especially yarns of regenerated cellulose filaments made by stretching cellulose ester yarns very substantially

2

while in a softened condition, for example while they are under the influence of steam or hot water, and thereafter saponifying them substantially completely. By applying the oiling treatment to such materials a very great improvement indeed can be secured as regards the sheerness and other properties. For example where the hosiery has already been coloured as is usually the case the limited application of drying oil results in a considerable apparent deepening of colour so that to obtain a particular shade in the finished material a smaller proportion of dye can be employed than would otherwise be necessary. It is possible that the oiling treatment greatly reduces the surface reflection of light by the material. Further the oiled material shows less tendency to develop ladders than does the untreated material.

The desired effects can be obtained with quite small proportions of the drying oil, for example from 10 to 35% e. g. about 20 or 25% based on the weight of the material, can be used. Smaller or greater proportions can however be employed, for instance proportions as low as 10%. The proportions employed can be such as merely to coat the yarn of which the fabric is made and should not be sufficient to close the interstices of the fabric. To effect such closure a proportion of the order of 200% is usually necessary.

30 It is convenient to apply the drying oil to the hosiery or other textile material as a solution in a volatile solvent therefor. In this way uniform distribution of the oil throughout the textile material can be readily secured. Thus a solution of a drying oil in benzene and of about 10% strength by volume can be employed. The oil may also be applied as an aqueous emulsion.

If desired the application of the oil can be combined with the clarifying treatment referred to above and described in our co-pending U. S. application S. No. 621,378, the oil being applied in solution in the hydrophobe liquid used, in conjunction with water, to treat the materials.

Suitable solvents for the drying oil are aliphatic or aromatic hydrocarbons, for example the benzene mentioned above, toluene, xylene, solvent naphtha or light fractions of petroleum. Again halogenated hydrocarbons can be employed for example carbon tetrachloride or perchlorethylene.

45 50 Solutions of drying oils in these solvents are suitable for application to the materials whether used as part of the clarifying treatment described in our above mentioned co-pending application or whether applied in a separate operation after the clarifying treatment.

In place of drying oils other substances capable of yielding a water-insoluble film on the filaments of the textile material particularly such as are soluble in organic solvents and can be applied as solutions in hydrophobe organic liquids. Examples of such other substances are natural resins and synthetic resins of the alkyd type whether "oil-modified" or not, resins of the polyvinyl acetal type, and those obtained by alkylating urea formaldehyde condensation products or melamine formaldehyde condensation products. Again varnishes of the resin/drying oil type can be employed. These can be diluted with volatile organic liquid and applied in the same manner as the simple solutions of drying oils referred to above.

The new treatment is of especial value in the case of cellulose textiles whether of natural or regenerated cellulose. Thus it can be applied to cotton materials or to materials of yarns of cellulose regenerated from viscose or cuprammonium solutions of cellulose or obtained by saponification of cellulose ester yarns. It has been found of particular value in the case of textiles of filaments of high tenacity e. g. above 2 grams per denier, made by spinning viscose solutions or cuprammonium solutions of cellulose and stretching the filaments substantially when partially but not completely set or made by stretching cellulose acetate or other cellulose ester filaments in a softened condition for example under the influence of a hot aqueous medium, e. g. wet steam or hot water, and subsequently saponifying them substantially completely. The treatment can be applied to fabrics consisting wholly or in part of such stretched and saponified filaments. The process can, however, be applied to textile materials of filaments other than cellulose filaments e. g. to materials of natural silk or of cellulose acetate or other cellulose ester or ether filaments, including cellulose ester or ether filaments which have been stretched substantially while in a softened condition e. g. while under the influence of wet steam or hot water, and cellulose ester or ether filaments produced by a wet spinning process.

#### Example 1

Hosiery dyed in a medium tan shade and knitted from 65 denier yarn obtained by stretching cellulose acetate yarn to about 10 times its length in wet steam and thereafter saponifying it substantially completely is wetted with a mixture of 100 parts by volume of acetone with 10 parts by volume of water. The hosiery is then drained and steeped in benzene until the material appears clear therein. This may require a few hours. The hosiery is then dried and oiled by immersion in a mixture of 10 volumes of boiled linseed oil and 100 volumes of benzene. It is then squeezed so that it retains about 2½ times its weight of the oil solution and hung in a steam heated cupboard at 75-85° C. for about 24 hours. The result is a considerable increase in the sheerness of the hose and a great improvement as regards uniformity of appearance. Further the colour appears much deeper than in the untreated hose. These properties are not materially affected by scouring for 15 minutes in a 5 gram per litre soap solution at 65° C.

#### Example 2

Dyed hosiery of the kind referred to in Example 1 is subjected to the same clarifying treatment as that described in that example and is then impregnated with a solution containing 10 grams of the thermoplastic resin sold by I. C. I. under the

trade name "Bedafin 285 X" per 100 ccs. of benzene. After squeezing, the material is dried, the results being very similar to those obtained according to Example 1.

5

#### Example 3

Dyed hosiery knitted from normal 75 denier 20 filament cellulose acetate yarn (i. e. dry spun yarn which has not been subjected to substantial stretching after spinning) is immersed in a mixture of 10 volumes of boiled linseed oil and 100 volumes of benzene. It is then squeezed and dried as in Example 1. The sheerness is thereby increased, the colour rendered more intense, and the tendency to ladder reduced.

Having described our invention, what we desire to secure by Letters Patent is:

1. Process of imparting sheerness and uniformity of appearance to hosiery of textile filaments made by stretching cellulose ester filaments while in a softened condition and saponifying them substantially completely, which comprises wetting the hosiery with an aqueous liquid and subjecting it while moist with water, to the action of a hydrophobe organic liquid selected from the group consisting of benzene, toluene, xylene, solvent naphtha, light fractions of petroleum, carbon tetrachloride, perchloroethylene and methylcyclohexanol until it appears clear therein and then uniformly impregnating it with from 10% to 35% of its weight of a drying oil and causing the latter to dry without closing the interstices in said hosiery.

2. Process of imparting sheerness and uniformity of appearance to hosiery of textile filaments made by stretching cellulose acetate filaments while in a softened condition and saponifying them substantially completely, which comprises wetting the hosiery with an aqueous liquid and subjecting it while moist with water, to the action of a hydrophobe organic liquid selected from the group consisting of benzene, toluene, xylene, solvent naphtha, light fractions of petroleum, carbon tetrachloride, perchloroethylene and methylcyclohexanol until it appears clear therein and then uniformly impregnating it with a solution of a drying oil in a volatile organic liquid so that the hosiery carries from 10% to 35% of its weight of drying oil and causing the latter to dry without closing the interstices in said hosiery.

3. Process of imparting sheerness and uniformity of appearance to hosiery of textile filaments made by stretching cellulose acetate filaments while in a softened condition and saponifying them substantially completely, which comprises wetting the hosiery with an aqueous liquid and subjecting it while moist with water, to the action of benzene until it appears clear therein and then uniformly impregnating it with from 10% to 35% of its weight of a drying oil and causing the latter to dry without closing the interstices in said hosiery.

4. Process according to claim 1, wherein the hosiery is knitted from yarns of filaments made by stretching cellulose ester yarns under the influence of a hot aqueous medium and thereafter saponifying them substantially completely.

5. Process for increasing the sheerness of hosiery knitted from yarns of filaments made by stretching cellulose ester yarns under the influence of a hot aqueous medium and thereafter saponifying them substantially completely, which comprises damping the hosiery with water, steeping it in benzene until it appears clear therein, and then impregnating it with a benzene solution

of boiled linseed oil and evaporating off the benzene so as to leave on the hosiery about 25 percent of its weight of the linseed oil without closing the interstices in said hosiery.

ALBERT MELLOR.

RALPH JAMES MANN.

DONALD FINLAYSON.

ALBERT WILLIAM MORLEDGE-HADFIELD.

#### REFERENCES CITED

10

The following references are of record in the file of this patent:

#### UNITED STATES PATENTS

| Number    | Name     | Date           |
|-----------|----------|----------------|
| 138,302   | Wagner   | Apr. 29, 1873  |
| 217,604   | Francis  | July 15, 1879  |
| 682,367   | Rosell   | Sept. 10, 1901 |
| 1,236,959 | McIntosh | Aug. 14, 1917  |

| Number    | Name      | Date          |
|-----------|-----------|---------------|
| 1,277,695 | Cavanaugh | Sept. 3, 1918 |
| 2,036,424 | Malm      | Apr. 7, 1936  |
| 2,053,766 | Dreyfus   | Sept. 8, 1936 |
| 2,075,887 | Dreyfus   | Apr. 6, 1937  |
| 2,137,404 | Hollerer  | Nov. 22, 1938 |
| 2,177,425 | Barker    | Oct. 24, 1939 |
| 2,192,919 | Kress     | Mar. 12, 1940 |
| 2,352,747 | Whitehead | July 4, 1944  |

#### FOREIGN PATENTS

| Number  | Country       | Date          |
|---------|---------------|---------------|
| 359,819 | Great Britain | Oct. 29, 1931 |
| 620,627 | Germany       | Oct. 24, 1935 |

#### OTHER REFERENCES

Randolph, Eliminating Bubbles in Fabric Impregnation C. & M. E. 35 306 (No. 5).